

## UNITED STATES PATENT OFFICE.

HYMAN STEIN, OF ARVERNE, WILLIAM E. AUSTIN, OF NEW YORK, AND IRVING LIEBOWITZ, OF BROOKLYN, NEW YORK, ASSIGNORS TO STEIN FUR DYEING CO. INC., OF NEW YORK, N. Y., A CORPORATION OF NEW YORK.

## BLEACHED AND DYED FURS AND THE LIKE.

No Drawing.

Application filed May 3, 1924. Serial No. 710,830.

To all whom it may concern:

Be it known that we, HYMAN STEIN, WILLIAM E. AUSTIN, and IRVING LIEBOWITZ, citizens of the United States, residing, respectively, in Arverne, Queens County, city and State of New York, in the borough of the Bronx, Bronx County, city and State of New York, and in the borough of Brooklyn, Kings County, city and State of New York, have invented an Improvement in Bleached and Dyed Furs and the like, of which the following is a specification.

Our present invention relates to fibrous materials, particularly of animal origin, such as fur skins and the like, and more particularly such products in a condition which renders them remarkably well suited and adapted to be bleached with little or no impairment of their strength, texture and lustre. Our invention relating also to the bleached and dyed products themselves. It is an object of the present invention to provide articles of the general character designated above which shall be in a condition admirably adapting them for their subsequent conversion into bleached and dyed products, and also to provide the bleached products in a remarkably fine condition as to lightness of color, but without loss of strength or impairment of their lustre and texture, the strength, lustre and texture of the bleached and dyed skins of the present invention being even improved, in certain cases, as compared with the skins dyed by the usual processes.

In the accompanying specification we shall describe an illustrative embodiment of the article of the present invention. It is, however, to be clearly understood that our invention is not limited to the specific embodiment thereof herein described for purposes of illustration only. In the accompanying specification we shall also describe a method of producing the article of the present invention, which method, however, is more fully described and is claimed in our copending application filed by us of even date herewith and entitled "Processes of

bleaching and dyeing furs and the like," Serial No. 710,829.

The article of the present invention, in its unbleached condition, in which condition, however, it is admirably adapted and suited for the subsequent bleaching operation, which operation may be carried out on such article without destroying or even impairing its strength, texture and lustre, is characterized by incorporating in the voids or interstices of the fibres of the fur skin or like article a "protective" agent. By a "protective" agent we mean, in the present instance, an agent which, while permitting the desired bleaching or decolorizing operation to be carried out efficiently and even with remarkable rapidity, protects the fibres of the fur skin or equivalent article from any destructive or weakening action of the bleaching agent. Such protective agents are preferably of mineral origin and preferably comprise reducing agents, such as ferrous compounds. An example of a protective agent which we have found particularly useful is ferrous sulphate.

The product, in its unbleached condition, may be obtained by soaking the fur skin or the like, preferably after it has previously been washed or "killed" by treatment for from about two to about three hours in an alkaline solution, such as a solution of sodium carbonate, in a solution of the protective agent, as in an aqueous solution containing from about 0.5 to about 5.0% crystallized ferrous sulphate, by weight. Since the protective agent is generally a reducing agent which would tend to become oxidized by exposure to the air, we prefer to add to the solution of the protective agent a stabilizing agent, which, in the case where the protective agent comprises a ferrous salt, such as ferrous sulphate, preferably consists of ammonium chloride added in an amount approximately equal to the ferrous sulphate used and equal to from about 0.5 to about 5.0 per cent, by weight. The fur skin or the like is soaked in the solution of the protective agent, with or without the added stabi-

lizing agent, overnight, or from about eight to about twelve hours.

By this treatment the voids or interstices of the skin become filled with the solution of the protective agent, which may or may not contain the stabilizing agent. After this treatment the skins are rinsed and hydro-extracted. It will therefore be noted that the skins treated with the solution of the protective agent contain such agent in the inner voids or interstices of the fibres of the skin or the like, rather than merely on the surfaces of such fibres. This is of great importance since it is one of the factors, in our opinion, although we do not wish to be limited to any particular theory or explanation of why the results of the present invention are obtained, which enables the subsequent bleaching operation to be carried out with little or no impairment of the strength of the fibres and of their fine lustre and texture.

The unbleached product described above is characterized by its remarkable adaptability to the subsequent bleaching operation, which operation may be carried out by the use of any suitable bleaching agent, but preferably by the use of hydrogen peroxide, or of sodium peroxide or sodium perborate, which latter are capable of yielding hydrogen peroxide in solution in the presence of liberating agents, generally of an acid character. Not only may the bleaching operation be conducted without impairment of the strength of the fibres or of their texture or lustre, but instead of requiring from about 24 to 72 hours, as had been the case previously for obtaining even the imperfect and unsatisfactory products of the bleaching processes as hitherto practiced, the unbleached product of the present invention described above requires only a fraction of this time for its proper and completely satisfactory bleaching.

The bleached product is characterized by the remarkable strength of the leather, and the remarkable strength, fine texture and lustre of the hair of the fur skin or the like. Such strength, lustre and texture compare very favorably with those of the natural skin and with those of the skins dyed to the desired color by applying merely the ordinary fur dyeing processes to the natural white or light colored skins. The bleached skin of the present invention will contain in its voids or interstices the protective agent which has, however, by this time been converted from a lower to a higher state of oxidation by the hydrogen peroxide or equivalent oxidizing bleaching agent. At the same time the pigment or color originally present in the fur skin will have been removed, in whole or in part, without, however, destroying or even impairing the strength, texture and lustre of the skin.

The bleached product described above may now be dyed to any light or other suitable color, hitherto obtainable only by dyeing natural white or light colored skins, by dyeing such skins in accordance with the usual dyeing processes customarily employed either for natural white or light colored skins, and with or without the use of a mordant. The dyed skins are characterized by their great strength and remarkably fine texture and lustre. The strength, texture and lustre, as well as the general appearance, of the dyed skins of the present invention are such as to render it difficult for all but experts, and often even for experts, to distinguish the dyed skins of the present invention from the dyed natural white or light colored skins as hitherto manufactured and sold. The dyed product of the present invention can therefore be sold at a price comparing favorably with the price of the dyed natural white or light colored skins, while costing much less, since it is manufactured from the comparatively cheap dark colored skin.

While the process for making the product of the present invention is more fully described and claimed in our copending application referred to above, it may be desirable, for the sake of a complete and full disclosure in the present case, to briefly summarize one specific illustrative example of the process, it being understood that the process is of general application and is not limited to the specific embodiment thereof herein described for purposes of example merely:

Brown moufflons are washed or "killed" in an alkaline solution, for example, a solution of sodium carbonate. This washing operation ordinarily requires from about 2 to about 3 hours. The washed or "killed" skins are then rinsed and thoroughly hydro-extracted. The skins are then immersed in a solution of the protective agent, such as in a solution of ferrous sulphate, and there allowed to remain over night. While the strength of the ferrous sulphate solution or its equivalent may vary within considerable limits, we prefer to use an aqueous solution of ferrous sulphate of a strength of from about 0.5 to 5.0 per cent of the solid crystallized ferrous sulphate, by weight. Such a solution may or may not contain the stabilizing agent. If a stabilizing agent, such as ammonium chloride, is used, we prefer to use it in an amount approximately proportionate to the amount of ferrous sulphate used and equalling from about 0.5 to about 5.0 per cent of ammonium chloride, by weight.

The fur skins or the like, after having been soaked for from about 8 to about 12 hours in the solution of the protective agent, with or without the addition of the stabiliz-

111 ing agent, are then rinsed and hydro-extracted. The treatment apparently impregnates or fills the voids and interstices of the fibres with the solution of protective agent. The 5 fur skins thus treated are now immersed in a solution of hydrogen peroxide or equivalent bleaching agent. However, in place of hydrogen peroxide, we may use other bleaching agents, particularly sodium per- 10 oxide or sodium perborate, which yield hydrogen peroxide in solution in the presence of certain liberating agents, generally of an acid character. The amount of hydrogen peroxide used may vary from about five 15 (5.0) to about one hundred (100.0) per cent by volume of a three (3.0) per cent solution of hydrogen peroxide. We prefer that the temperature at which the bleaching or decolorizing operation is carried out 20 shall be between 60° and 100° F.

The skins are subjected to the action of the bleaching or decolorizing agent until they have been sufficiently decolorized. The bleached or decolorized skins are then rinsed 25 and can, if desired, be dyed directly in accordance with any of the well known or desirable processes employed for dyeing furs or the like. We may, however, subject the bleached or decolorized skins to the usual 30 dyeing operations of washing and mordanting, and then dyeing the washed and mordanted skins in accordance with the practice hitherto generally employed for dyeing furs.

The advantages and superiorities of the 35 product of the present invention in its various stages—unbleached, bleached, and dyed—are numerous and of great practical importance, and may be briefly summarized as follows: The unbleached product, which 40 may be sold as such and sent to any bleachery for bleaching furs in accordance with the principles of the present invention, is characterized by containing in its pores, voids or interstices, a protective agent, with or without a stabilizing agent, and being thus admirably suited and adapted for the bleaching operation. By means of the 45 presence of the protective agent, with or without the stabilizing agent, in the fibres of the fur skin or the like, the bleaching operation may be conducted simply, conveniently, economically and very expeditiously, requiring only a fraction of the time hitherto required for the imperfect and 50 unsatisfactory bleaching processes as customarily practiced. It may here be stated that while the protective agent, with or without the stabilizing agent, protects the fibres from destructive action of the bleaching agent, it 55 at the same time greatly accelerates the desired bleaching action.

The bleached, but undyed, skin is characterized by its great strength and by its remarkably fine texture and lustre, and contains in its interstices the protective agent,

by this time raised from a lower to a higher state of oxidation by the action of the hydrogen peroxide or other oxidizing bleaching agent. The bleached skin will be found to be remarkably well adapted to be subjected 70 to the subsequent dyeing operation, which dyeing operation may be conducted with or without the use of a mordant.

The dyed product is characterized by having the strength, texture, lustre and appearance of the dyed natural white or light colored skin. For this reason, the dyed skin finds a wide and ready market and a ready sale at a price much greater than the dyed dark colored skin would fetch in the market 80 and at a price comparing very favorably with the price of the dyed natural white or light colored skins.

It may here be stated that in addition to the mineral protective agent, such as the ferrous sulphate, with or without the addition of the stabilizing agent, the solution for giving the fur skins or the like their protective treatment for the subsequent bleaching operation may contain other compatible metal 90 salts, as well as suitable protective colloids, such as glue, gelatin, or the like, generally in relatively small amounts. It may here also be stated that the method described above may be applied with almost equal 95 success in the treatment of skins which have already been dyed, either a dark or a light color, and whether satisfactorily or not, but preferably skins which have been dyed by the use of a mordant consisting of a ferrous 100 compound, such as ferrous sulphate, or an equivalent substance, thus producing from the previously dyed skins the superior product described above.

What we claim as our invention is:

1. As an article of manufacture, an unbleached fur skin or the like suitable for bleaching and being impregnated with a solution of a protecting agent to protect the skin against harmful oxidation during a 110 subsequent bleaching operation.

2. As an article of manufacture, an unbleached fur skin or the like suitable for bleaching and being impregnated with a solution of a mineral reducing agent.

3. As an article of manufacture, an unbleached fur skin or the like suitable for bleaching and being impregnated with a solution of a ferrous salt.

4. As an article of manufacture, an unbleached fur skin or the like suitable for bleaching and being impregnated with a solution of a mineral reducing agent to which has been added a stabilizing agent.

5. As an article of manufacture, an unbleached fur skin or the like suitable for bleaching and being impregnated with a solution of a ferrous salt to which has been added a stabilizing agent.

6. As an article of manufacture, an un-

- bleached fur skin or the like suitable for bleaching and being impregnated with a solution of a protecting agent to which has been added an agent for stabilizing the protecting agent to protect the skin against harmful oxidation during a subsequent bleaching operation.
7. As an article of manufacture, an unbleached fur skin or the like adapted for bleaching and containing in its fibres a mineral reducing agent.
8. As an article of manufacture, an unbleached fur skin or the like adapted for bleaching and containing in its fibres a ferrous compound.
9. As an article of manufacture, an unbleached fur skin or the like adapted for bleaching and containing in its fibres a mineral reducing agent and a stabilizing agent.
10. As an article of manufacture, an unbleached fur skin or the like adapted for bleaching and containing in its fibres a ferrous compound and ammonium chloride.
11. As an article of manufacture, a bleached fur skin or the like the fibres of which contain a protecting agent converted from a lower to a higher state of oxidation by the bleaching agent, said protecting agent having served to protect the skin from harmful oxidation under the action of said bleaching agent.
12. As an article of manufacture, a bleached fur skin or the like the fibres of which contain a mineral protecting agent converted from a lower to a higher state of oxidation by the bleaching agent, said protecting agent having served to protect the skin from harmful oxidation under the action of said bleaching agent.
13. As an article of manufacture, a bleached fur skin or the like the fibres of which contain a mineral protecting agent in the form of an iron compound converted from the ferrous to the ferric state of oxidation by the bleaching agent, said protecting agent having served to protect the skin from harmful oxidation under the action of said bleaching agent.
14. As an article of manufacture, a bleached fur skin or the like the fibres of which contain a mineral protecting agent converted from a lower to a higher state of oxidation by hydrogen peroxide, said protecting agent having served to protect said skin from excessive oxidation under the action of the hydrogen peroxide.
15. As an article of manufacture, a bleached fur skin or the like the fibres of which contain a mineral protecting agent in the form of an iron compound converted from the ferrous to the ferric state of oxidation by hydrogen peroxide, said protecting agent having served to protect said skin from excessive oxidation under the action of the hydrogen peroxide.
16. As an article of manufacture, a bleached fur skin or the like the fibres of which contain a protecting agent converted from a lower to a higher state of oxidation by hydrogen peroxide, said protecting agent having served to protect said skin from excessive oxidation under the action of the hydrogen peroxide.
17. As an article of manufacture, a bleached and dyed fur skin or the like having the fibres of the leather and hair making up the fur skin or the like substantially unimpaired as to strength, texture and lustre.
18. As an article of manufacture, a bleached and dyed fur skin or the like having the fibres of the leather and hair making up the fur skin or the like substantially unimpaired as to strength, texture and lustre and containing an iron compound raised from a lower to a higher state of oxidation by the bleaching agent before the fur skin or the like has been dyed.
19. As an article of manufacture, a bleached and dyed fur skin or the like having the fibres of the leather and hair making up the fur skin or the like substantially unimpaired as to strength, texture and lustre and containing an iron compound raised from a lower to a higher state of oxidation by the hydrogen peroxide or other bleaching agent before the fur skin or the like has been dyed.
20. As an article of manufacture, a bleached and dyed fur skin or the like having the fibres of the leather and hair making up the fur skin or the like substantially unimpaired as to strength, texture and lustre, and having the appearance, feel and texture of a fur skin or the like of the same species dyed to the same color from the natural white or other light colored fur skin or the like.
21. As an article of manufacture, an unbleached fur skin or the like suitable for bleaching and being impregnated with a mineral protecting agent to protect the skin against harmful chemical action during a subsequent bleaching operation.
22. As an article of manufacture, an unbleached fur skin or the like suitable for bleaching and being impregnated with a mineral protecting agent to which has been added an agent for stabilizing the protecting agent to protect the skin against harmful chemical action during a subsequent bleaching operation.
23. As an article of manufacture, a bleached and dyed fur skin or the like containing the dye stuff in combination with a metallic protecting compound raised from a lower to a higher state of oxidation by the hydrogen peroxide or other bleaching agent before the fur skin or the like has been dyed, said protecting compound having served to

protect the skin against harmful chemical action during the bleaching operation.

24. As an article of manufacture, a bleached and dyed fur skin or the like containing the dye stuff in combination with a metallic protecting compound raised from a lower to a higher state of oxidation by the bleaching agent before the fur skin or the like has been dyed, said protecting com-

pound having served to protect the skin <sup>10</sup> against harmful chemical action during the bleaching operation.

In testimony whereof, we have signed our names to this specification this 23rd day of April, 1924.

HYMAN STEIN.

WILLIAM E. AUSTIN.

IRVING LIEBOWITZ.

### DISCLAIMER

1,564,378.—*Hyman Stein, Arverne, William E. Austin, New York, and Irving Liebowitz, Brooklyn, N. Y. BLEACHED AND DYED FURS AND THE LIKE.* Patent Dated December 8, 1925. Disclaimer filed May 3, 1933, by the assignee, *Steinfur Patents Corporation*.

Hereby enters this disclaimer to that part of the claims in said specification which is in the following words, to wit:

“17. As an article of manufacture, a bleached and dyed fur skin or the like having the fibres of the leather and hair making up the fur skin or the like substantially unimpaired as to strength, texture and lustre.”

“20. As an article of manufacture, a bleached and dyed fur skin or the like having the fibres of the leather and hair making up the fur skin or the like substantially unimpaired as to strength, texture and lustre, and having the appearance, feel and texture of a fur skin or the like of the same species dyed to the same color from the natural white or other light colored fur skin or the like.”

[Official Gazette May 30, 1933.]